# EUROPEAN PATENT SPECIFICATION

(11) **EP 2 803 423 B1**
(45) Date of publication and mention of the grant of the patent: **07.06.2023**
(21) Application number: 13717409.0
(22) Date of filing: 04.02.2013
(51) Int. Cl.: B21C 1/24, B22D 11/00, C22C 9/00

(54) **COPPER TUBE FOR THE CONSTRUCTION INDUSTRY AND PROCESS FOR PREPARING IT**
KUPFER-ROHR FÜR DIE BAUINDUSTRIE UND DESSEN HERSTELLUNGSVERFAHREN
TUBE EN CUIVRE POUR L'INDUSTRIE DE LA CONSTRUCTION ET SON PROCÉDÉ DE FABRICATION

(43) Date of publication of application: 19.11.2014
(73) Proprietor: La Farga Tub, S.L., 08509 Les Masies de Voltregà Barcelona (ES)
(72) Inventor: MOREL RODRÍGUEZ, Eduardo Andrés, Las Condes Santiago (CL); VALDEBENITO LÓPEZ, Eduardo Alfonso, La Florida Santiago (CL); CARRASCO GÁLVEZ, Marco Antonio, Puente Alto Santiago (CL)
(74) Representative: Isern Patentes y Marcas S.L.
(86) International application number: PCT/CL2013/000007
(87) International publication number: WO 2014/117285

(56) References cited:
- EP-A2- 2 055 795
- WO-A1-01/64372
- WO-A2-2008/072787
- US-A- 4 876 870
- US-A- 5 279 353
- US-A- 6 106 764
- UPCAST OY: "New UPCAST Developments Target Copper Tube Production and Environmental Benefits", TECHNOLOGY NEWS INTERNATIONAL 99/2010, 2010, pages 28-29, XP002755545,

## Description

### TRADITIONAL PROCEDURE

The traditional process generally commences with the melting of material with which cylinders, commonly known as "billets" (technical term), are cast in a range of 9.8 cm (3.5 inches) and 25.4 cm (10 inches) or more. Then these billets are heated at high temperatures to later be extruded in a high-pressure press, or perforated and lengthened by means of mechanical systems whose result is what is known in the industry as "pre-tube" which, as we pointed out, will be referred to in this specification as "old pre-tube". This old pre-tube has a length that is predetermined by the size and weight of the billet. In the industry, the weight of the billet currently oscillates between 75 and 400 kilos, which restricts the size of the old pre-tube because it must be limited to the capacity of the extrusion press or the perforators.

Once the old pre-tube is formed, it passes through a series of wiredrawing processes that consist, basically, of stretching and reducing the thickness of its walls by using traction to pass it through:
i. A tungsten carbide die;
ii. With a "plug" or "chuck" or "mandrel".
Both are shown in Figures 1 and 2.

In other words, the old system consists of passing a tube through a die or hollow plate whose hole has walls of tungsten carbide of a diameter smaller than the mentioned tube. The tube is threaded through said hole (after reducing its diameter at one end) and a plug or metallic cylinder with a diameter somewhat larger than the hole in the sheet is placed within the pre-tube. Thus, when traction is applied to the tube, the mentioned plug is pushed by the tube, locks and permits the reduction of the thickness of the wall while passing through the die, as shown in Figures 1 and 2. The execution of this process is necessary because the initial old pre-tube has a diameter larger than 60 mm, which requires that it be reduced until the commercial standardized measurements are reached. It is important to point out that not more than 30% of the tube's original dimension is reduced in each wiredrawing process. In view of the latter, the tube must necessarily be passed repeatedly through this wiredrawing process to reach the commercially required diameters. For example, the mass-produced end product, generally of a nominal 3/4 inch according to ASTM standard B-88, whose real diameter is 7/8 of an inch (22.22 mm) must pass through at least 10 processes to reach those diameters (Figure 4), which raises the cost of the process and, therefore, of the tube, especially due to the consumption of the following associated supplies:
- High energy expenditure,
- Unnecessary cost increase of materials,
- Labor intensive in excess, and
- Generating of cuttings of the old pre-tubes (or losses of material) that is produced for 3 reasons, mainly:
   - First, in order to thread the tube in the die (to make it pass through its hole) and thus be able to apply traction with regard to same, the size needs to be reduced (taper one end), deforming the first 30 or 40 cm of each tube each time it passes, which material is then lost.
   - The second source of loss is material breakage. As the diameter of the tube gets smaller, the tractions become more intense and the material accumulates stress deformation with each passing. If there is an imperfection in the tube, the tube breaks and produces a loss of material.
   - Finally, the third source of loss is the final dimensioning of the product that will depend directly on the length of the old pre-tube or the weight of the billet and the size required by the end customer.

In addition, other technologies are known in the state of the art, such as the one described in the patent application EP 2055795 which refers to a copper alloy tube for a heat exchanger, comprising Sn 0.1 to 2.0 mass%, P 0.005 to 0.1 mass%, S 0.005 mass% or less, O 0.005 mass% or less, and H 0.0002 mass% or less; and the remainder has a composition consisting of Cu and unavoidable impurities, wherein the copper alloy tube has the following characteristics: a tensile strength in the longitudinal direction of the copper alloy tube is 250 N/MM2 or more; an average grain diameter is 30 µm or less when measured in the direction perpendicular to the thickness direction of the tube, in the cross section perpendicular to the tube axis; and assuming that a tensile strength in the longitudinal direction of the copper alloy tube is σL, and a tensile strength in the circumferential direction of the same is σT, σT/σL> 0.93 holds.

Also, UPCAST OY, "New UPCAST Developments Target Copper Tube Production and Environmental Benefits", TECHNOLOGY NEWS INTERNATIONAL 99/2010, (2010), pages 28 - 29, discloses the UPCAST ^{®} - SG technology for producing thin walled copper tubes with desired grain size, comprising the steps of continuous vertical casting of a pre-tube, drawing of the pre-tube in 9 passes using spinning blocks, and carrying out an intermediate induction annealing for recrystallization of the cast grain structure.

### INNOVATIVE PROCESS OF THIS INVENTION

The production process of this invention consists of unifying in a three-stage production line to obtain a standardized tube that is equivalent to one eighth of the process of the traditional line. These can be seen in Figure 5.

The stages of this online production process will be described below:

### CONTINUOUS VERTICAL CASTING

The continuous vertical casting process is a process that was created in the nineteen seventies for the exclusive manufacture of oxygen free high conductivity (OFHC) wire rod.

During the month of May 2008, a failed casting occurred in one of these machines at Madeco that produced a continuous hollow wire rod. This continuous hollow wire rod, after multiple breakthroughs and tests, finally became the origin of patent application 1935-2011 and application PCT/CL2012/00013.

From that moment and to this date, different ways have been tried to obtain tubes from this type of casting machine. It has been possible to standardize the casting process in a pre-tube of 38 × 2.5 mm.

With regard to the operation of the casting machine, following is a description of the melting process and initiation of the casting.

An automatic loading machine feeds copper cathodes into the smelting furnace, where the melted metal is maintained at a temperature of 1160 ± 5 °C covered with a layer of graphite in flakes to partially avoid its oxidation.

Prior to starting the casting process, a special cooler is set up with a graphite matrix, a kaowool cup, a graphite cup and a mortar, all shown in Figure 7.

The casting process is started with the insertion of a steel tube ("fishing rod") with a piece of perforated steel on the tip (Figure 8). When this assembly is inserted in the liquid metal, the liquid metal enters the graphite matrix and solidifies on the perforated point, it is left to settle for a short time and then the fishing rod is pulled upward with the help of the traction machine and the pinch rolls ( Figure 9 and Figure 10 ), when the metal pre-tube has passed over the traction table the fishing rod is removed and its point cut ( Figure 11 ). At that moment, that pre-tube stands up by itself and is taken to the receivers where they are accumulated. Henceforth the mentioned pre-tubes made using this process will be called "new pre-tubes".

These new pre-tubes have two special characteristics that distinguish them from the old pre-tubes and that interfere with their reduction to marketable sizes. These are:
a. Their structural micro sequencing, of disorderly (depending on their cooling) and large size grains that produce:
   i. The fragility of that pre-tube in the wiredrawing process; and,
   ii. Easy appearance of micro fissures in the wiredrawing process; and
b. Their resulting rapid oxidation that produces the breakage of the pre-tube in the wiredrawing process due to the emanation of the particles of free oxides.

With the invention described in this process we have successfully resolved all the above-mentioned problems.

The materiality of the tube comprises copper.

One object of this disclosure is the sequence of additional steps required to ensure that the new pre-tube (just taken from the continuous vertical casting machine) can end up being a marketable product.

Another object of this disclosure is to obtain a tube in which the type of grain required for its application can be selected, which includes a tube with a minimum or no degree of oxidation.

Some characteristics of the tube of copper, obtained with the process that will be described below, are: that it has grains whose formation is equiaxial, with an average grain size of 0.03mm.

Moreover, chemically the copper tube has a sulfur concentration of 6.58 ppm and an oxygen concentration of 10.45 ppm.

With regard to the process proposed in this invention, the sequence of steps required will be indicated.

### WIREDRAWING PROCESS

As was commented with regard to the old system, the wiredrawing process consists, basically, of stretching and reducing the thickness of the walls of a tube by using traction to pass the tube through a tungsten carbide die with a plug or chuck or mandrel inside it until the desired result is achieved. In a disclosure, there are different ways in which to execute the wiredrawing process, as shown in Figures 2 and 3.

As disclosed herein, the type of wiredrawing for the new pre-tubes originating from the continuous vertical casting is the floating plug type indicated in Figure 2 mentioned previously.

As disclose herein, the new pre-tube is received from the continuous casting with measurements of 38.00 × 2.50 mm +/- 5%. It is then taken to the wiredrawing sector where a double wiredrawing process is carried out thanks to the joining and synchronization of two wiredrawing machines that work in tandem.

The material is prepared before starting the wiredrawing process. As disclosed herein, the new pre-tube is brought close to the jig borer where it is lubricated on the inside, a tungsten carbide plug is inserted ( Figure 1 ) and subsequently a point is made at the beginning of the rolled up tube, which is then inserted in a winder to start up the wiredrawing line at a constant speed using paraffin as an exterior lubricating/refrigerating agent. As disclosed herein, the new pre-tube passes through the first wiredrawing machine ( Figure 12 ), then through a stress regulator ( Figure 13 ), then the mentioned new pre-tube passes through the second wiredrawing machine ( Figure 14 ) that executes the second section reduction using the mentioned lubricant/coolant to finally accumulate the material in a receiver that is inserted in baskets ( Figure 15 ) in which the material is transferred to the following stage (annealing oven and cooling chamber).

### ANNEALING OVEN AND COOLING CHAMBER

As herein disclosed, the mechanical properties of the tube are recovered in this process (a re-crystallization of the tube takes place).

As herein disclosed, without this step it would be impossible to control the pre-tube's fragility in the wiredrawing process as the structural arrangement that it has enables the appearance of micro-fissures, as was said, disorderly and large size grains, and their attendant rapid oxidation that produces their breakage in the wiredrawing process due to the emanation of free oxide particles. The wiredrawing process cannot be carried out satisfactorily without solving those problems.

As herein disclosed, the material received from the wiredrawers is inserted manually into the inlet guides of the furnace (Figure 16).

As herein disclosed, to start the process, the inside of the new pre-tube is purged with nitrogen. It then enters a chamber where a solvent, such as turpentine, is applied to the exterior of the tube to remove the lubricant and other elements that affect the process such as dust, shavings or stains, among others. The tube then enters a furnace where induction coils are used to heat the metal. This furnace works at a maximum speed of preferably 40 meters/minute and a maximum current intensity of 5000 Amp. Subsequently the tube passes through a cooling chamber where the temperature of the metal is reduced to room temperature, to finally roll the tube inside a basket. Protective wax is applied during the passage to that zone

As herein disclosed, the zone of the furnace and cooling chamber are constantly saturated with purged nitrogen.

The final product is a tube with an equiaxial grain structure having an average size of 0.030 mm, a hardness of 35 HRF, a diameter of 28.2 × 1.9 mm, a phosphorous concentration of 0.024% wt, a sulfur concentration of 6.58 ppm, an arsenic concentration of 0.001% wt, an iron concentration of 0.001 % wt, a silver concentration of 0.001% wt, an oxygen concentration of 10.45 ppm, a Cu + Ag concentration of 99.970% wt and 0.000% wt of Zn, Ni, Pb, Sb, Bi, and Sn. Also, it is herein disclosed that as it is worked in an inert environment this avoids the forming of oxidation on the tube's surface, therefore the final product complies with the characteristics identified commercially.

In a particular embodiment, the process of the invention is addressed to preparing a copper tube for the construction industry, wherein said tube comprises equiaxial grains with a grain size of 0.03 mm, a hardness of 35 HRF, a diameter of 28.2 × 1.9 mm, a phosphorous concentration of 0.024% wt, a sulfur concentration of 6.58 ppm, an arsenic concentration of 0.001% wt, an iron concentration of 0.001 % wt, a silver concentration of 0.001% wt, an oxygen concentration of 10.45 ppm, a Cu + Ag concentration of 99.970% wt and 0.000% wt of Zn, Ni, Pb, Sb, Bi, and Sn, comprising
a) The pre-tube obtained from the continuous vertical casting process is prepared with the tapering equipment, the pre-tube is lubricated internally and a wiredrawing chuck is inserted. Then a point is made at the beginning of the roll of pre-tube and it is inserted in the spool.
b) The first wiredrawer is started up at a constant speed;
c) The tube that comes out of the first wiredrawer passes through tension regulating equipment in tandem;
d) The tube that has already passed through the first wiredrawer contained by the tension regulating equipment passes to the second wiredrawer also in tandem, where a second reduction is carried out;
e) The material that comes out of the second wiredrawer is accumulated continuously in baskets;
f) The material accumulated and that has passed through two wiredrawers enters the annealing furnace in order to realign the microstructure of the final tube reducing the oxidation speed so that it can be stranded;
g) The tube is purged internally with nitrogen;
h) The exterior of the tube is cleaned;
i) The furnace heats the tube by induction;
j) The tube quickly passes into a cooling chamber;
k) The final tube is rolled up in a basket for its subsequent dimensioning.

In another particular embodiment, the production process is CHARACTERIZED in that the input speed to the process comprises a maximum speed of the continuous vertical casting of 1 m/min, water flow of 50 L/min and a water pressure of 8 bar.

In another particular embodiment, the production process is CHARACTERIZED in that the raw material of the wiredrawers that work synchronized and in tandem is the pre-tubes produced in the continuous vertical casting, and a reduction is applied in the first reduction in the range of 30.25% to 38.38% preferably of 38.38% and in the second reduction in the range of 22.69% to 26.78% preferably 26.78%, achieving an accumulated reduction in the range of 46.08% to 54.88%, preferably of 54.88%.

In another particular embodiment, the production process is CHARACTERIZED in that the wiredrawers at points c) and e) work at an average speed of 35m/min and they also have a cooling system in each machine.

In another particular embodiment, the production process is CHARACTERIZED in that paraffin is used as an exterior lubricating/cooling agent.

In another particular embodiment, the production process is CHARACTERIZED in that the induction furnace works with the product of the wiredrawing machines at a speed preferably in the range of 6m/min - 40m/min, and with a power preferably in the range of 1200 - 5000 A. In another particular embodiment the solvent used in point h) is preferably turpentine prior to entering the furnace as just described and with protective wax between the cooling zone and the coiling zone. In another particular embodiment, the induction furnace as just described works at a speed of 40m/min preferably with a power of 600 Kva.

Once the process is known, these are the principal advantages that the tube manufacturing process using continuous vertical casting has versus the traditional procedures:
1. It increases productivity because the size of the lot of the continuous vertical casting line is twenty times higher than the traditional procedure (1500 kg vs. 75 kg respectively), which optimizes the use of energy in approximately 18%, losses of material in approximately 40%.
2. It does not require prior melting for the manufacture of the cylinders as the line has its own small smelting works. This reduces the consumption of energy and the pollutant emissions of a traditional melting process as the metal is heated by induction.
3. It permits the obtaining of tubes of different sizes and especially of a smaller diameter in a shorter time in the termination process. This is a very important characteristic in relation to energy consumption and losses of material because less processing steps are required to arrive at the end product.
4. Being able to start off with pre-tubes having smaller diameters makes it possible to arrive at smaller diameter tubes with greater safety and quality as the melt has been exposed to less stress. In the best of cases, the percentage of reprocessing in the traditional system reaches 25%; with the vertical continuous casting process and the process that is the object of this patent it is possible to reach a 5% of reprocessing.
5. The final tube that passed through the vertical continuous casting process differs in the chemical composition shown in the following table I, in which a diminution in the amount of S and O₂ can be appreciated.

| Table I. Maximum impurities | | | | | | | | | | | | | |
|---|---|---|---|---|---|---|---|---|---|---|---|---|---|
| Proces s | P | S | As | Zn | Ni | Fe | Pb | Sb | Bi | Ag | Sn | O | Cu+ Ag |
| | % | pp m | % | % | % | % | % | % | % | % | % | pp m | % |
| C1220 0 | 0.01 5-0.03 0 | 60 | 0.0 20 | 0.0 15 | 0.0 25 | 0.0 12 | 0.0 05 | 0.0 05 | 0.0 02 | - | 0.0 05 | 70 | 99.9 min |
| Inventi on | 0.02 4 | 6.5 8 | 0.0 01 | 0.0 00 | 0.0 00 | 0.0 01 | 0.0 00 | 0.0 00 | 0.0 00 | 0.0 01 | 0.0 00 | 10. 45 | 99.9 70 |
| Traditi onal | 0.02 0 | 13. 39 | 0.0 01 | 0.0 01 | 0.0 01 | 0.0 01 | 0.0 01 | 0.0 00 | 0.0 00 | 0.0 01 | 0.0 00 | 51. 73 | 99.9 72 |

6. The processing time of 1000 kg by way of continuous vertical casting for a 3/4L product is 45% faster than the traditional process.
7. The personnel required for the production of the continuous vertical casting is 35% lower than that used in the traditional process.
8. The type of grain with which one wants to materialize the tube can be selected.

Comparatively, the tube itself, obtained via the process described in this invention, is very different to the products in the processes of the prior state of the art.

These physical characteristics can be analyzed on the basis of the following table II:

| Table II | | | | |
|---|---|---|---|---|
| Process | Tube (mm) | Grain size (mm) | Hardness HRF | Comments |
| Traditional process Piercing | 85 x 8 | 0.09 | 81 | Equiaxial non homogenous grains |
| Pre-tube vertical casting | 38 x 2.5 | 0.461 x 0.206 | 53 | With columnar non homogenous grains |
| Invention | 28.2 x 1.9 | 0.03 | 35 | Homogenous equiaxial grains |

From an analysis of Table II, it is clear that grain distribution for the process of this invention is highly homogeneous, which reduces the speed of oxidation and deterioration of the tube. The rest of the tests are part of the state of the art where non homogenous grains and/or macrograins are obtained with large spaces where the oxygen penetrates and increases the variability in their distribution generating numerous spaces, thus making oxygen penetration easier.

The combination of grain size and hardness provide better mechanical properties for tube production to the end consumer.

Finally, the pre-tube is presented in the penultimate line, which corresponds to the development closest to this invention and the last line of the table corresponds to the innovative system with the application of this patent.

### DESCRIPTION OF FIGURES:

Figure 1.
   (1) Dies
   (2) Plugs
Figure 2.
   (1) Dies
   (2) Plugs
   (3) Pre-tube
Figure 3.
   (1) Dies
   (3) Fixed mandrel
   (4) Pre-tube
Figure 4.
   (5) Traditional process
   (5a) Smelting
   (5b) Piercing or rotary pressure system
   (5c) Pickling
   (5d) Taperer 1
   (5e) Bench 120,000 lbs.
   (5f) Taperer 2
   (5g) Bench 50,000 lbs.
   (5h) Bull Block 10,000 lbs.
   (7) Cutting process
Figure 5.
   (6) Continuous vertical casting process
   (6a) Continuous melting
   (6b) Wiredrawing in tandem
   (6c) Annealing
   (6d) Spinner
   (7) Cutting process
Figure 6
   (5) Traditional process
   (5a) Smelting
   (5b) Piercing or rotary pressure system
   (5c) Pickling
   (5d) Taperer 1
   (5e) Bench 120,000 lbs.
   (5f) Taperer 2
   (5g) Bench 50,000 lbs.
   (5h) Bull Block 10,000 lbs.
   (6) Continuous vertical casting process
   (6a) Continuous melting
   (6b) Wiredrawing in tandem
   (6c) Annealing
   (6d) Spinner
   (7) Cutting process
Figure 7
Figure 8
   (8) Squeeze rollers
   (9) Traction rollers
   (10) Fishing tube
   (11) Cooling water
   (12) Furnace
   (13) Kaowool sleeve
   (14) Fishing point
   (15) Graphite cup
   (16) Liquid copper
   (17) Graphite matrix
Figure 9.
   (14) Fishing point
   (18) New pre-tube
   (19) Solidification front
Figure 10.
   (14) Fishing point
   (18) New pre-tube
   (19) Solidification front
Figure 11.
   (18) New pre-tube
   (19) Solidification front
Figure 12.
Figure 13.
Figure 14.
Figure 15.
Figure 16.
Figure 17.
Figure 18. Comparative micrographs of the products obtained in the different processes of the state of the art and the current process of the invention.
   (20) Section of a copper pipe with large size, non-uniform grains, with spaces for the oxidation, of the continuous vertical casting process with the annealing process known in the state of the art.
   (21) Section of a copper pipe with macro grains, segregation, with ample space for the oxidation, of the classic processes known in the state of the art, without the continuous casting system.
   (22) Section of a copper pipe with homogeneous formation of grains, with minimum segregation and minimum spaces for the oxidation, of the process of this invention subsequent to the formation of the new pre-tube by the continuous casting.

### EXAMPLE OF APPLICATION

As an example of application, which is not according to the invention, we shall bear in mind the manufacture of a nominal 3/4 inch standard tube for the construction industry.

Once 1300-1500 kilograms of the new pre-tube have been melted and cast through the continuous vertical casting, these are taken to the wiredrawing process section for a first and second wiredrawing in two wiredrawing machines working synchronously until a tube with a diameter of preferably 30.00 × 1.44 mm is reached.

The product of these wiredrawing machines is accumulated in a basket as shown in Figure 15 that links the wiredrawing process with the annealing process.

After being annealed, the material is processed in a circular wiredrawer giving a single wiredrawing undercut, and finally, the finishing undercut in the straight wiredrawers.

Comparatively, in the traditional process for the same nominal 3/4 inch tube for the construction industry, mentioned in the previous example, the flowchart of this process can be appreciated in Figure 4. In that traditional process, the tube was extruded initially or was obtained by means of a mechanical process as was mentioned previously. Then, as the tube became hot and deformed, it needed to be manipulated to clean it of all impurities or traces of oxide. For the latter, a process known as "pickling" is executed that consists of a chemical bath to remove these impurities. Once the tube is clean, the point is made so that it can be stranded. Once this has been done, the tube is taken to the wiredrawing banks; these banks, where the tube is stretched, are approximately 30 to 40 meters long.

Once the initial reduction is carried out on the banks and a tube is produced that has a diameter close to the one desired, the tube passes to a wiredrawing process in rollers using circular wiredrawing machines. These have the same function as the banks but with smaller diameters and longer tubes. Once the desired diameter and thickness have been reached, the tube is cut in the lengths required commercially.

## Claims

1. A process for preparing a copper tube for the construction industry, wherein said tube comprises equiaxial grains with a grain size of 0.03 mm, a hardness of 35 HRF, a diameter of 28.2 × 1.9 mm, a phosphorous concentration of 0.024% wt, a sulfur concentration of 6.58 ppm, an arsenic concentration of 0.001% wt, an iron concentration of 0.001 % wt, a silver concentration of 0.001% wt, an oxygen concentration of 10.45 ppm, a Cu + Ag concentration of 99.970% wt and 0.000% wt of Zn, Ni, Pb, Sb, Bi, and Sn, comprising:
a) A pre-tube obtained from a continuous vertical casting process is prepared with the tapering equipment, the pre-tube is lubricated internally and a wiredrawing chuck is inserted. Then a point is made at the beginning of the roll of pre-tube and it is inserted in the spool.
b) The first wiredrawer is started up at a constant speed;
c) The tube that comes out of the first wiredrawer passes through tension regulating equipment in tandem;
d) The tube that has already passed through the first wiredrawer contained by the tension regulating equipment passes to the second wiredrawer also in tandem, where a second reduction is carried out;
e) The material that comes out of the second wiredrawer is accumulated continuously in baskets;
f) The material accumulated and that has passed through two wiredrawers enters the annealing furnace in order to realign the microstructure of the final tube reducing the oxidation speed so that it can be stranded;
g) The tube is purged internally with nitrogen;
h) The exterior of the tube is cleaned;
i) The furnace heats the tube by induction;
j) The tube quickly passes into a cooling chamber;
k) The final tube is rolled up in a basket for its subsequent dimensioning.

2. A production process in accordance with claim 1, **CHARACTERIZED in that** the input speed to the process comprises a maximum speed of the continuous vertical casting of 1 m/min, water flow of 50 L/min and a water pressure of 8 bar.

3. A production process in accordance with claim 1, **CHARACTERIZED in that** the raw material of the wiredrawers that work synchronized and in tandem is the pre-tubes produced in the continuous vertical casting, and a reduction is applied in the first reduction in the range of 30.25% to 38.38% preferably of 38.38% and in the second reduction in the range of 22.69% to 26.78% preferably 26.78%, achieving an accumulated reduction in the range of 46.08% to 54.88%, preferably of 54.88%.

4. A production process in accordance with claim 1, **CHARACTERIZED in that** the wiredrawers at points c) and e) work at an average speed of 35m/min and they also have a cooling system in each machine.

5. A production process in accordance with claim 4, **CHARACTERIZED in that** paraffin is used as an exterior lubricating/cooling agent.

6. A production process in accordance with claim 1, **CHARACTERIZED in that** the induction furnace works with the product of the wiredrawing machines at a speed preferably in the range of 6m/min - 40m/min, and with a power preferably in the range of 1200 - 5000 A.

7. A production process in accordance with claim 6, **CHARACTERIZED in that** the induction furnace works at a speed of 40m/min preferably with a power of 600 Kva.

8. A production process in accordance with claim 6, **CHARACTERIZED in that** the solvent used in point h) is preferably turpentine prior to entering the furnace and with protective wax between the cooling zone and the coiling zone.

9. A copper tube for the construction industry comprising equiaxial grains with a grain size of 0.03 mm, a hardness of 35 HRF, a diameter of 28.2 × 1.9 mm, a phosphorous concentration of 0.024% wt, a sulfur concentration of 6.58 ppm, an arsenic concentration of 0.001% wt, an iron concentration of 0.001% wt, a silver concentration of 0.001% wt, an oxygen concentration of 10.45 ppm, a Cu + Ag concentration of 99.970% wt and 0.000% wt of Zn, Ni, Pb, Sb, Bi, and Sn, wherein said tube is obtained by the process according to claim 1.

## Patentansprüche

1. Verfahren zur Präparierung eines Kupferrohrs für die Bauindustrie, wobei das Rohr gleichachsige Körner mit einer Korngröße von 0,03 mm, einer Härte von 35 HRF, einem Durchmesser von 28,2 × 1,9 mm, einer Phosphorkonzentration von 0,024 Gew.-%, einer Schwefelkonzentration von 6,58 ppm, einer Arsenkonzentration von 0,001 % Gew.-%, einer Eisenkonzentration von 0,001 % Gew.-%, einer Silberkonzentration von 0,001 % Gew-%., einer Sauerstoffkonzentration von 10,45 ppm, einer Cu-Ag-Konzentration von 99,970 % Gew.-% und 0,000 Gew.-% Zn, Ni, Pb, Sb, Bi und Sn, umfassend:
a) ein aus einem vertikalen Stranggussverfahren erhaltenes Vorrohr wird mit der Verjüngungsvorrichtung präpariert, das Vorrohr wird innen geschmiert und ein Drahtziehfutter wird eingesetzt. Dann wird am Anfang des Rollens des Vorrohrs eine Spitze angebracht und in die Spule eingeführt.
b) Der erste Drahtzieher wird mit konstanter Geschwindigkeit angefahren;
c) Das Rohr, das aus dem ersten Drahtzieher kommt, durchläuft im Tandem die Spannungsregulierungsvorrichtung;
d) Das Rohr, das bereits den ersten Drahtzieher durchlaufen hat, der von der Spannungsregulierungsvorrichtung umfasst ist, wird auch im Tandem zum zweiten Drahtzieher geführt, wo eine zweite Reduzierung durchgeführt wird;
e) Das Material, das aus dem zweiten Drahtzieher kommt, wird kontinuierlich in Körben gesammelt;
f) Das angesammelte Material, das zwei Drahtzieher durchlaufen hat, tritt in den Glühofen ein, um die Mikrostruktur des fertigen Rohrs neu auszurichten, wodurch die Oxidationsgeschwindigkeit reduziert wird, damit es verseilt werden kann;
g) Das Rohr wird innen mit Stickstoff gespült;
h) Das Äußere des Rohrs wird gereinigt;
i) Der Ofen erwärmt das Rohr durch Induktion;
j) Das Rohr gelangt schnell in eine Kühlkammer;
k) Das fertige Rohr wird zur späteren Dimensionierung in einem Korb aufgerollt.

2. Herstellungsverfahren nach Anspruch 1, **dadurch gekennzeichnet, dass** die Eingangsgeschwindigkeit in das Verfahren eine maximale Geschwindigkeit des vertikalen Stranggusses von 1 m/min, einen Wasserfluss von 50 l/min und einen Wasserdruck von 8 bar umfasst.

3. Herstellungsverfahren nach Anspruch 1, **dadurch gekennzeichnet, dass** das Rohmaterial der synchron und im Tandem arbeitenden Drahtzieher die im vertikalen Strangguß hergestellten Vorrohre sind und bei der ersten Reduktion eine Reduktion im Bereich von 30,25 % bis 38,38 %, vorzugsweise 38,38 %, und bei der zweiten Reduktion im Bereich von 22,69 % bis 26,78 %, vorzugsweise 26,78 %, angewendet wird, wodurch eine kumulierte Reduzierung im Bereich von 46,08 % bis 54,88 %, vorzugsweise 54,88 %, erreicht wird.

4. Herstellungsverfahren nach Anspruch 1, **dadurch gekennzeichnet, dass** die Drahtzieher an den Punkten c) und e) mit einer Durchschnittsgeschwindigkeit von 35 m/min arbeiten und außerdem ein Kühlsystem in jeder Maschine aufweisen.

5. Herstellungsverfahren nach Anspruch 4, **dadurch gekennzeichnet, dass** als äußeres Schmier-/Kühlmittel Paraffin verwendet wird.

6. Herstellungsverfahren nach Anspruch 1, **dadurch gekennzeichnet, dass** der Induktionsofen mit dem Produkt der Drahtziehmaschinen mit einer Geschwindigkeit vorzugsweise im Bereich von 6 m/min - 40 m/min und mit einer Leistung vorzugsweise im Bereich von 1200 - 5000 A arbeitet.

7. Herstellungsverfahren nach Anspruch 6, **dadurch gekennzeichnet, dass** der Induktionsofen mit einer Geschwindigkeit von 40 m/min vorzugsweise mit einer Leistung von 600 Kva arbeitet.

8. Herstellungsverfahren nach Anspruch 6, **dadurch gekennzeichnet, dass** das in Punkt h) verwendete Lösungsmittel vorzugsweise Terpentin vor dem Eintritt in den Ofen und mit Schutzwachs zwischen der Kühlzone und der Aufwickelzone ist.

9. Kupferrohr für die Bauindustrie, umfassend gleichachsige Körner mit einer Korngröße von 0,03 mm, einer Härte von 35 HRF, einem Durchmesser von 28,2 × 1,9 mm, einer Phosphorkonzentration von 0,024 Gew.-%, einer Schwefelkonzentration von 6,58 ppm, einer Arsenkonzentration von 0,001 Gew.-%, einer Eisenkonzentration von 0,001 Gew.-%, einer Silberkonzentration von 0,001 Gew.-%, einer Sauerstoffkonzentration von 10,45 ppm, einer Cu-Ag-Konzentration von 99,970 Gew.-% und 0,000 Gew.-% Zn, Ni, Pb, Sb, Bi und Sn, wobei das Rohr durch das Verfahren nach Anspruch 1 erhalten wird.

## Revendications

1. Procédé de préparation d'un tube en cuivre pour l'industrie du bâtiment, dans lequel ledit tube comprend des grains équiaxiaux d'une granulométrie de 0,03 mm, une dureté de 35 HRF, un diamètre de 28,2 × 1,9 mm, une concentration en phosphore de 0,024 % en poids, une concentration en soufre de 6,58 ppm, une concentration en arsenic de 0,001 % en poids, une concentration en fer de 0,001 % en poids, une concentration en argent de 0,001 % en poids, une concentration en oxygène de 10,45 ppm, une concentration en Cu + Ag de 99,970 % en poids et 0,000 % en poids de Zn, Ni, Pb, Sb, Bi, et Sn, comprenant :
a) Un prétube obtenu à partir d'un procédé de coulée verticale continue est préparé avec l'équipement de délardage, le prétube est lubrifié intérieurement et un mandrin de tréfilage est inséré. Puis une pointe est fabriquée au début du rouleau de prétube et elle est insérée dans la bobine.
b) La première tréfileuse est mise en marche à une vitesse constante ;
c) Le tube qui sort de la première tréfileuse passe à travers un équipement régulateur de tension en tandem ;
d) Le tube qui est déjà passé à travers la première tréfileuse contenue par l'équipement régulateur de tension passe jusqu'à la seconde tréfileuse également en tandem, où une seconde réduction est effectuée ;
e) Le matériau qui sort de la seconde tréfileuse est accumulé en continu dans des paniers ;
f) Le matériau accumulé et qui est passé à travers deux tréfileuses entre dans le four de recuit afin de réaligner la microstructure du tube final en réduisant la vitesse d'oxydation de manière à ce qu'il puisse être toronné ;
g) Le tube est purgé intérieurement avec de l'azote ;
h) L'extérieur du tube est nettoyé ;
i) Le four chauffe le tube par induction ;
j) Le tube passe rapidement dans une chambre de refroidissement ;
k) Le tube final est enroulé dans un panier pour son dimensionnement ultérieur.

2. Procédé de production selon la revendication 1, **CARACTÉRISÉ en ce que** la vitesse d'entrée jusqu'au procédé comprend une vitesse maximale de la coulée verticale continue de 1 m/min, un débit d'eau de 50 L/min et une pression d'eau de 8 bar.

3. Procédé de production selon la revendication 1, **CARACTÉRISÉ en ce que** le matériau brut des tréfileuses qui fonctionnent de manière synchronisée et en tandem est les prétubes produits dans la coulée verticale continue, et une réduction est appliquée dans la première réduction dans la plage de 30,25 % à 38,38 % de préférence de 38,38 % et dans la seconde réduction dans la plage de 22,69 % à 26,78 % de préférence 26,78 %, atteignant une réduction accumulée dans la plage de 46,08 % à 54,88 %, de préférence de 54,88 %.

4. Procédé de production selon la revendication 1, **CARACTÉRISÉ en ce que** les tréfileuses au niveau des points c) et e) fonctionnent à une vitesse moyenne de 35 m/min et elles ont également un système de refroidissement dans chaque machine.

5. Procédé de production selon la revendication 4, **CARACTÉRISÉ en ce que** la paraffine est utilisée comme agent de lubrification/refroidissement extérieur.

6. Procédé de production selon la revendication 1, **CARACTÉRISÉ en ce que** le four à induction fonctionne avec le produit des machines de tréfilage à une vitesse de préférence dans la plage de 6 m/min à 40 m/min, et avec une puissance de préférence dans la plage de 1 200 à 5 000 A.

7. Procédé de production selon la revendication 6, **CARACTÉRISÉ en ce que** le four à induction fonctionne à une vitesse de 40 m/min de préférence avec une puissance de 600 kVA.

8. Procédé de production selon la revendication 6, **CARACTÉRISÉ en ce que** le solvant utilisé au point h) est de préférence de la térébenthine avant l'entrée dans le four et avec de la cire protectrice entre la zone de refroidissement et la zone de bobinage.

9. Tube en cuivre pour l'industrie du bâtiment comprenant des grains équiaxiaux d'une granulométrie de 0,03 mm, une dureté de 35 HRF, un diamètre de 28,2 × 1,9 mm, une concentration en phosphore de 0,024 % en poids, une concentration en soufre de 6,58 ppm, une concentration en arsenic de 0,001 % en poids, une concentration en fer de 0,001 % en poids, une concentration en argent de 0,001 % en poids, une concentration en oxygène de 10,45 ppm, une concentration en Cu + Ag de 99,970 % en poids et 0,000 % en poids de Zn, Ni, Pb, Sb, Bi, et Sn, dans lequel ledit tube est obtenu par le procédé selon la revendication 1.
